

## 1

3,275,402

## FORMALDEHYDE MODIFICATION OF CELLULOSE CONDUCTED IN THE PRESENCE OF A STIFFENING AGENT AND A LEWIS ACID METALLIC SALT

George C. Daul and Thomas F. Drake, Mobile, and Marshall W. Duke, Daphne, Ala., assignors, by mesne assignments, to Courtaulds, Limited, London, England, a British company

No Drawing. Filed June 2, 1961, Ser. No. 114,313

15 Claims. (Cl. 8—115.6)

This application relates to a process for improving the properties of cellulosic textile materials and especially to a process for imparting permanent wash-wear properties to said materials.

The demand for wash-wear fabrics has increased greatly in recent years. Broadly speaking, wash-wear fabrics are those which after washing and drying by conventional methods, recover or retain an ironed appearance without pressing. An index to the wash-wear properties of a given fabric is its "crease recovery angle," as defined in ASTM Designation: D1295-53T.

Various processes have been proposed for imparting suitable crease recovery properties to cellulosic textiles. In the copending application of Daul and Drake, Serial No. 81,956, filed January 11, 1961 (which is a continuation-in-part of applications Serial Nos. 51,781, filed August 25, 1960, 38,418, filed June 24, 1960, and 792,696, filed February 12, 1959), there is described a process for cross linking cellulose with formaldehyde using as the curing agent a metallic salt which is a Lewis acid in the solid state. Preferably the formaldehyde and curing agent are applied at pH 5 or above. By means of this process it is possible to cross link the cellulose with relatively little adverse effect on its physical properties, especially its tensile strength, a drawback which had blocked widespread use of prior formaldehyde processes.

Cellulosic textiles treated according to the above process have improved dry crease recovery properties, i.e. when washed and allowed to "drip-dry," in an unrumpled state they assume a fresh, ironed appearance. However, unless the amount of formaldehyde bound to the fiber is very great, good wet crease recovery properties cannot be obtained, i.e. if washed and "spun-dried" so that they are dried in a rumpled state, they will not present an ironed appearance. Since many homes are equipped with mechanical driers it is important that clothes be "spin-dryable" and to get this effect both wet and dry crease recovery properties must be imparted.

This problem has not gone unrecognized and several solutions have been offered to overcome it. One of these involves treating the cellulose with formaldehyde and a strong acid so that reaction is effected while the fabric is wet. Another process involves impregnating the fabric with an aqueous solution of dichloropropanol and then storing the fabric for an extended time in a closed container. These processes are awkward to employ industrially, use expensive reagents and in some cases cause very serious damage to the textile material.

From very early times the properties of textiles have been modified by applying stiffening agents. Starch is probably the oldest of such materials but many more easily spring to mind. Conventionally these stiffeners have been used for temporary effects which are lost in large measure after a single wash. It has been suggested that their permanency can be enhanced by applying them in the presence of formaldehyde. However, in such processes the treating conditions have been such that the amount of formaldehyde bound to the fabric was less than that necessary for improved crease recovery.

## 2

It has now been found that the wet crease recovery of a fabric is a function of the dry stiffness of the fabric and that by applying any of the well known stiffeners which are capable of reacting with formaldehyde, to a cellulose fabric and applying formaldehyde to the fabric using the technique described in the Daul et al. applications mentioned above, it is possible to obtain fabrics having excellent wet and dry crease recovery properties, thus meeting both major requirements for wash-wear textiles.

The invention accordingly envisions a method for imparting wet and dry crease recovery properties to cellulosic textiles which comprises impregnating said textiles with formaldehyde, with at least 0.0030 mol, per 100 g. of cellulose, of a curing agent which is a metallic salt and a Lewis acid in the solid state and which is water soluble to the extent of at least 0.03 mol per liter at 20° C. and pH 5, and a polymeric film forming stiffening material capable of reacting with formaldehyde, said impregnation with formaldehyde and metallic salt being effected in the presence of water at a pH of at least 5, and curing the impregnated material to cross link the cellulose and to bind the film forming material to the cellulose.

The invention can be applied to any variety of cellulosic fabrics, woven fabrics, knitted fabrics, the so-called "no-woven" fabrics or even paper. The fabrics may consist wholly of cellulose fiber or in part of cellulose fibers and in part of fibers of other kinds, for example, cellulose acetate (acetone-soluble cellulose acetate or cellulose triacetate) fibers, fibers of synthetic linear polymers, for example of polyamides, such as nylon 6 or nylon 66, fibers of polyesters, for example polyethylene terephthalate, or fibers of addition polymers derived from acrylonitrile. Preferably when blends are treated, the cellulose fibers comprise at least 35% by weight of the blend.

If desired, the cellulose, prior to treating, may have been dyed with any one of many common dyes, without adverse effect.

The formaldehyde used may be added to the treating solution as the normal 40% aqueous commercial solution. Other sources, e.g. paraformaldehyde, may, however, be used as desired.

As noted above, the curing agent should be a metallic salt which is a Lewis acid.

In determining whether any given salt is a Lewis acid, the procedure described by Walling, JACS 72, pp. 1164-1168 and Pines and Haag, JACS, 82, pp. 2471-2483, may be used. A particularly suitable test is to take a small quantity of the salt, dried to remove surface moisture, and allow it to stand overnight with a solution of the leuco base of Malachite Green (4,4-di(dimethylamino)-triphenyl methane) in a dry, non-polar solvent such as cyclohexane or isoctane. The development of a green color at the salt surface indicates that the salt is a Lewis acid. An alternative test may be based on the response of a compound to an indicator such as Methyl Red (whose range in aqueous solution is pH 4.4-6.2) under the conditions described by Walling (72 JACS, 1164). Indicators such as Methyl Red have the drawback of giving positive reactions in the presence of traces of acid (in the classical sense). On the other hand, the Malachite Green leuco base reaction appears to be inhibited by traces of classical acids.

In addition to being a Lewis acid, the curing agent should preferably be soluble and form no precipitate in aqueous solution at pH 5 at concentrations of at least 0.03 mol/liter at 20° C. For reasons explained more fully below, solutions at pH 6 or above are highly desirable for cotton and, therefore, when cotton is to be treated, the curing agent should be soluble at that pH. Salts which remain soluble at higher pH are, of course, more advantageous. Obviously, salts which are highly

colored or highly toxic or become so during the process are undesirable.

Salts which meet these qualifications are in general those in which the metal is bivalent and belongs to Group II of the periodic table and the acid radical is that of a strong monobasic acid which is at least 50% ionized in normal aqueous solution at 18° C., such as hydrochloric, hydrobromic, hydriodic, nitric, perchloric and thiocyanic acids. Of most interest are salts of calcium, magnesium, strontium, barium and zinc. Examples of suitable salts would include  $\text{CaCl}_2$ ,  $\text{CaBr}_2$ ,  $\text{CaI}_2$ ,  $\text{Ca}(\text{NO}_3)_2$ ,  $\text{Ca}(\text{SCN})_2$ ,  $\text{Mg}(\text{NO}_3)_2$ ,  $\text{MgCl}_2$ ,  $\text{MgBr}_2$ ,  $\text{Mg}(\text{ClO}_4)_2$ ,  $\text{MgI}_2$ ,  $\text{ZnCl}_2$ , and  $\text{Zn}(\text{NO}_3)_2$  as well as  $\text{SrCl}_2$ ,  $\text{BaCl}_2$ , and  $\text{CdCl}_2$ .  $\text{ZnSO}_4$  may also be employed. Either the anhydrous salt or a hydrate may be used, as may mixtures of salts. Generally the magnesium salts are preferred as being less acidic (in the classical sense) than the zinc salts and more effective (as curing agents) than the other salts mentioned. The magnesium halides are especially favored and of these, magnesium chloride is outstanding.

Magnesium chloride is of exceptional value in the present process for several reasons. First, it is stable in solutions with formaldehyde at pH up to about 9. This enables even the most sensitive cellulose material to be impregnated and dried with minimal damage. Moreover, magnesium chloride has a very pronounced effect in lowering the vapor pressure of formaldehyde, possibly as the result of a complex formation. This tends to prevent loss of formaldehyde during curing, increasing the efficiency of the process.

The stiffeners which may be employed in the present invention include virtually all stiffeners employed in the textile industry, provided they are capable of reaction with formaldehyde. They are in general organic film forming polymeric materials having one or more reactive hydroxyl ( $-\text{OH}$ ) or amino ( $-\text{NH}_2$ ) groups per molecule. A list of such stiffeners would include starch, starch derivatives such as hydroxyethyl starch, carboxymethyl starch, oxidized starches, hydrolysed starches and chemically modified starches such as acylated starches and alkylated starches. The list would further include dextran, dextran derivatives, dextrin, gelatin, natural gums of various sorts such as gum arabic, gum tragacanth, and locust bean gum, casein, soybean protein, albumin and algin. Synthetic stiffeners are also useful, such as polyvinyl alcohol, polyacrylamide, cellulose derivatives including ethers such as hydroxyethyl cellulose, methyl cellulose and carboxy methyl cellulose. Certain water-soluble vinyl ethers may also be used such as polyvinyl methyl ether.

The manner in which the formaldehyde and stiffeners are applied to the fabric is not especially important provided that the stiffener is deposited on the fabric before the formaldehyde-cellulose reaction is perfected. Whatever technique is used to apply the formaldehyde, catalyst and stiffener to the fabric, it is essential that at least 0.03 mol of curing agent, per 100 g. of cellulose is deposited on the fabric and preferably between about 0.10 and about 0.45 mol, per 100 g. of cellulose. Sufficient formaldehyde is deposited so that after drying and curing between about 0.1 and about 3.0%, preferably between about 0.4 and about 3.0%, based on cellulose, is chemically bound to the cellulose.

The amount of stiffener deposited is normally in the range of 0.25 to 10.0% on the weight of cellulose.

Conveniently the formaldehyde, curing agent and stiffener are applied from aqueous solutions. One solution may be used for all of the treating agents, but in some instances it may be desirable to apply one or more of the formaldehyde, curing agent and stiffener in a separate solution. The solution or solutions may contain solvents other than water such as methanol or ethanol, but should contain at least 10% by weight water.

The concentration of formaldehyde in the treating solution may vary to a considerable extent depending on

whether natural or regenerated cellulose is treated and on the structure of the fabric.

In general, it has been found that the amount of curing agent deposited on the fiber and the efficiency of the curing agent in reacting unbound formaldehyde with cellulose are more significant than the concentration of formaldehyde in the solution, provided that enough formaldehyde is present during curing to furnish the desired quantity of formaldehyde required to be bound to the cellulose for the particular physical properties sought. An overall range of recommended concentrations would extend from about 0.5 to about 8.0% by weight. Rayon fabric will normally require 1.0 to 8.0%, cotton fabric 0.5 to 4.0% by weight. It will be understood that higher concentrations may be employed, but serve no useful purpose. Indeed, it is one of the advantages of the present application that relatively dilute formaldehyde solutions can be used. Such solutions are less apt to lose formaldehyde by evaporation and are easier to work with from the point of view of operator health and comfort than the more concentrated solutions prescribed in many prior processes.

The concentration of curing agent may vary considerably, depending on the agent. Normally it will be between about 0.03 and about 0.90 g. mol/liter; preferably between about 0.1 and about 0.45 g. mol/liter. However, it is the proportion of curing agent deposited on the fiber and to the extent that the minimum amount of formaldehyde must be present during curing, the molar ratio of agent to formaldehyde, which is significant.

The pH of the solution will depend on the material being treated. Natural cellulose, such as cotton, is generally more sensitive to acid degradation and therefore when cotton is to be treated, a higher pH must be used than is necessary with regenerated cellulose. Generally the treating solution pH should not be less than 5 for regenerated cellulose and not less than 6 for cotton.

Some of the salts listed above when put into water with formaldehyde at use concentrations will not give pH's in this range. When used in the present invention they are, therefore, preferably buffered, for example, with sodium carbonate, sodium bicarbonate, or sodium hydroxide, to a pH of at least 5, or at least 6 if cotton is to be treated.

While the upper pH limit is not especially critical, some of the salts most useful with the present invention will form precipitates at pH's above about 10.

The temperature of the treating solution is not especially significant. Room temperature is satisfactory, although lower temperatures may be used to prevent loss of formaldehyde. Normally, temperatures of say 15° C. to 50° C. are used.

The concentration of stiffener may vary from say 0.25% to 10.0% by weight. Again it is the amount of stiffener applied to the fabric rather than the concentration in the treating solution which is important.

The actual manipulative techniques used in applying the solution or solutions to the fabric may be any of these well known to the art, e.g. padding or spraying. Following application of the liquor the fabric is usually squeezed to remove excess liquor and to maintain between say 120% and 50% of liquor (based on the weight of bone dry unimpregnated fabric) on the fabric.

Following impregnation, the material is dried at say 30-110° C. for whatever time is required to reduce the moisture content to say 5% by weight of the bone dry material, and then cured by heating to temperatures from about 110° C. to about 180° C. for periods which may range from say 30 minutes to a few (say about 5) seconds.

The temperatures and time for curing must be carefully selected, having in mind the pH at which the treatment has been conducted and the curing agent used. Thus, where a pH of 5 has been used, curing must be conducted under mild conditions within the range set forth, i.e. if a high temperature is used, a very short time should be used, or if a long time is used, the temperature should be

low, within the range set forth. If more rigorous curing conditions are employed, and the impregnation was at a low pH, there is danger of tendering the material.

By their nature most Lewis acids are capable of forming hydrates and since the present treatment involves application of aqueous solutions, the curing agent is normally deposited as a hydrate. With most salts at least a part of the hydrate water is evolved during curing. It has been found that during this water evolution the cellulose-formaldehyde reaction is inhibited or at least markedly depressed. To avoid such inhibition or depression it is therefore desirable to conduct the curing at temperatures either above, below or between the range or ranges at which the particular curing agent used loses large amounts of water of hydration.

Since it is desirable to conduct curing as expeditiously as possible temperatures below dehydration temperature are not usually employed. At the same time extremely high temperatures are to be avoided for fear of damage to the cellulose.

Because of these factors, salts which are Lewis acids and which can be heated at intermediate temperatures without water evolution are extremely desirable as curing agents, other things being equal. One of the properties that makes magnesium chloride especially attractive as a curing agent in the present process is that although it loses some water at about 120° C., there is an intermediate temperature range in which comparatively little water is evolved and the compound can therefore function effectively as a curing agent without a prolonged curing time or an excessively high temperature.

Zinc salts are generally more likely to cause degradation than, say, magnesium salts and greater care must be exercised in curing when the agent is a zinc compound.

As the pH of the treatment is increased, more rigorous curing conditions may be used, within the range set forth, without adversely affecting the properties of the material.

Obviously the drying and curing steps may be combined in a single treatment, if desired.

Fabric treated in accordance with the invention is characterized by a much firmer hand than untreated fabric and this firmness is permanent to washing. Moreover, it has improved crease recovery properties in both the wet and dry states with respect to untreated fabric. Normally the wet crease recovery angle is from 50 to 150° higher and the dry crease recovery angle from 10 to 70° higher than those of untreated fabric. While the physical properties, such as tensile strength, may in some instances be less than that of untreated fabric, this decrease is that which always accompanies cross-linking and is not due to a weakening or tendering of the individual fibers such as would occur with prior formaldehyde treatments. The cellulose chains are cross linked as indicated by the water

purposes of illustration only and are not to be taken as in any way restricting the invention beyond the scope of the appended claims.

*Example 1*

5 This example illustrates a technique which may be used to determine whether or not a given salt is a Lewis acid capable of cross-linking cellulose.

The leuco base of Malachite Green is purified by repeated recrystallization from absolute methanol until the solid gives no green color when dissolved in glacial acetic acid. A 0.5% by weight solution of the purified base in pure cyclohexane is then prepared.

15 Approximately 5-10 grams of the salt to be tested is spread on a shallow dish and placed in a moving air stream at 80° C. for about 30 minutes. A small portion, say 0.5 g. of the dried salt is then placed in a test tube and 2 to 3 ml. of the leuco base-cyclohexane solution is added to the tube. The mixture is allowed to stand for 12 hours. The development of a green color on the surface of the salt at the salt-liquid interface indicates that 20 the salt is a Lewis acid.

25 The results obtained with this test on a few salts are listed in Table I below. In the table "positive" means that a green color developed.

TABLE I

| Salt:                                            | Reaction  |
|--------------------------------------------------|-----------|
| MgCl <sub>2</sub> ·6H <sub>2</sub> O             | Positive. |
| Al <sub>2</sub> (SO <sub>4</sub> ) <sub>2</sub>  | Do.       |
| Zn(NO <sub>3</sub> ) <sub>2</sub>                | Do.       |
| CuSO <sub>4</sub>                                | Do.       |
| CaCl <sub>2</sub>                                | Do.       |
| (NH <sub>4</sub> ) <sub>2</sub> SO <sub>4</sub>  | Negative. |
| (NH <sub>4</sub> ) <sub>2</sub> HPO <sub>4</sub> | Do.       |

Similar results can be obtained using a 0.1% solution of Methyl Red in isooctane in place of the Malachite Green leuco base solution.

Care should be taken to see that prior to testing the salts are dried to remove surface water, since this will interfere with the above tests. For example, if CaCl<sub>2</sub> or MgSO<sub>4</sub>·7H<sub>2</sub>O are permitted to stand in the air for several hours and tested without drying, they will give no color. Yet if properly dried, as outlined above, they will give a positive test and, with proper curing temperatures, 40 can be made to promote the formaldehyde-cellulose reaction.

*Example 2*

50 Samples of rayon fabric were treated with aqueous solutions at pH 7 containing varying amounts of formaldehyde, MgCl<sub>2</sub>·6H<sub>2</sub>O, and starch, squeezed to about 100% pickup, frame dried at 80° C. for 10 minutes, cured at 160° C. for 5 minutes, washed and dried. The samples were then tested for water imbibition, formaldehyde content and crease recovery angle, dry and wet. Results appear in Table II.

TABLE II

| Sample           | Deposition (Percent Wt. of Fabric) |                                      |      | Mols<br>MgCl <sub>2</sub> ·6H <sub>2</sub> O<br>per 100 g.<br>Cell. | Fabric Properties        |                         |     |                        |      |
|------------------|------------------------------------|--------------------------------------|------|---------------------------------------------------------------------|--------------------------|-------------------------|-----|------------------------|------|
|                  | Starch                             | MgCl <sub>2</sub> ·6H <sub>2</sub> O | HCHO |                                                                     | Percent<br>Bound<br>HCHO | CRA° (W+F) <sup>2</sup> |     | Stiffness <sup>3</sup> |      |
|                  |                                    |                                      |      |                                                                     |                          | Dry                     | Wet |                        |      |
| 1-----           | 0.5                                | 5.5                                  | 5.55 | 0.0271                                                              | 1.00                     | 40.2                    | 231 | 261                    | 0.98 |
| 2-----           | 1.0                                | 5.5                                  | 5.55 | 0.0271                                                              | 2.20                     | 41.0                    | 227 | 275                    | 1.05 |
| 3-----           | 2.5                                | 5.5                                  | 5.55 | 0.0271                                                              | 1.76                     | 39.9                    | 233 | 260                    | 1.14 |
| 4 (Control)----- |                                    |                                      |      |                                                                     |                          |                         | 195 | 145                    | 0.50 |

<sup>1</sup> WI% = Water imbibition, percent. See Journal of the Society of Dyers and Colourists, Oct. 1948, p. 331.

<sup>2</sup> CRA° (W+F) = Crease recovery Angle (Warp & Filling). See ASTM Designation: D1295-53T.

<sup>3</sup> Stiffness = Pierce Bending Length (inches). See ASTM Designation: D1388-53T.

imbibition which is normally on the order of 35 to 60% and by the insolubility of the cellulose, after treatment, in cuprammonium hydroxide.

The invention will be further described with reference to the following specific examples which are given for 75

*Example 3*

The procedure of Example 2 was followed using various proportions of gelatin instead of starch. Results are shown in Table III.

TABLE III

| Sample | Deposition (Percent Wt. of Fabric) |                                      |      | Mols<br>MgCl <sub>2</sub> .6H <sub>2</sub> O<br>per 100 g.<br>Cell. | Fabric Properties        |      |            |     |           |
|--------|------------------------------------|--------------------------------------|------|---------------------------------------------------------------------|--------------------------|------|------------|-----|-----------|
|        | Gelatin                            | MgCl <sub>2</sub> .6H <sub>2</sub> O | HCHO |                                                                     | Percent<br>Bound<br>HCHO | WI%  | CRA° (W+F) |     | Stiffness |
|        |                                    |                                      |      |                                                                     |                          |      | Dry        | Wet |           |
| 1      | 1.0                                | 5.5                                  | 5.55 | 0.0271                                                              | 2.20                     | 39.9 | 206        | 271 | 1.52      |
| 2      | 1.0                                | 5.5                                  | 7.40 | 0.0271                                                              | 2.60                     | 37.8 | 243        | 273 | 1.35      |
| 3      | 2.5                                | 5.5                                  | 5.55 | 0.0271                                                              | 1.59                     | 43.1 | 203        | 273 | 1.50      |

## Example 4

The procedure of Example 1 was repeated using polyacrylamide. Results are shown in Table IV.

To demonstrate the laundering stability of finishes according to the invention, swatches of rayon fabric proc-

TABLE IV

| Sample | Deposition (Percent Wt. of Fabric) |                                      |      | Mols<br>MgCl <sub>2</sub> .6H <sub>2</sub> O<br>per 100 g.<br>Cell | Fabric Properties        |      |            |     |           |
|--------|------------------------------------|--------------------------------------|------|--------------------------------------------------------------------|--------------------------|------|------------|-----|-----------|
|        | Poly-<br>acryl-<br>amide           | MgCl <sub>2</sub> .6H <sub>2</sub> O | HCHO |                                                                    | Percent<br>Bound<br>HCHO | WI%  | CRA° (W+F) |     | Stiffness |
|        |                                    |                                      |      |                                                                    |                          |      | Dry        | Wet |           |
| 1      | 0.5                                | 4.5                                  | 1.85 | 0.0222                                                             | 0.72                     | 51.3 | 175        | 240 | 1.23      |
| 2      | 0.5                                | 5.5                                  | 5.55 | 0.0271                                                             | 2.10                     | 37.8 | 217        | 252 | 1.08      |
| 3      | 1.0                                | 5.5                                  | 5.55 | 0.0271                                                             | 2.30                     | 39.4 | 211        | 274 | 1.39      |
| 4      | 2.0                                | 4.5                                  | 1.85 | 0.0222                                                             | 0.92                     | 50.9 | 164        | 270 | 1.81      |
| 5      | 2.0                                | 5.5                                  | 5.55 | 0.0271                                                             | 1.30                     | 44.0 | 200        | 284 | 1.88      |
| 6      | 4.0                                | 5.5                                  | 5.55 | 0.0271                                                             | 1.70                     | 48.5 | 168        | 289 | 2.13      |

## Example 5

The procedure of Example 1 was repeated using polyvinyl alcohol. The results are shown in Table V. A consideration of Table V will show that polyvinylalcohol being somewhat more flexible and elastic than, for example, starch, does not give as high a stiffness as starch and will not impart as high a wet crease recovery angle

as starch. 35 essed in accordance with the invention were washed with Tide detergent for 10 cycles in a Frigidaire home washer. The stiffness (bending length) was measured after the first, fifth and tenth wash and compared with the bending length before washing. For the sake of further comparison, the same amount of stiffener was applied with-

TABLE V

| Sample | Deposition (Percent Wt. of Fabric) |                                      |      | Mols<br>MgCl <sub>2</sub> .6H <sub>2</sub> O<br>per 100 g.<br>Cell | Fabric Properties        |      |            |     |           |
|--------|------------------------------------|--------------------------------------|------|--------------------------------------------------------------------|--------------------------|------|------------|-----|-----------|
|        | PVA                                | MgCl <sub>2</sub> .6H <sub>2</sub> O | HCHO |                                                                    | Percent<br>Bound<br>HCHO | WI%  | CRA° (W+F) |     | Stiffness |
|        |                                    |                                      |      |                                                                    |                          |      | Dry        | Wet |           |
| 1      | 2.5                                | 4.5                                  | 1.85 | 0.0222                                                             | 0.59                     | 52.5 | 192        | 217 | 0.55      |
| 2      | 2.5                                | 5.5                                  | 3.70 | 0.0271                                                             | 0.93                     | 52.9 | 200        | 227 | 0.55      |
| 3      | 2.5                                | 5.5                                  | 5.55 | 0.0271                                                             | 1.61                     | 40.9 | 219        | 242 | 0.65      |
| 4      | 2.5                                | 5.5                                  | 7.40 | 0.0271                                                             | 1.98                     | 36.6 | 226        | 261 | 0.65      |

## Example 6

The procedure of Example 1 was repeated using di-

aldehyde starch. The results are reported in Table VI. 60 out formaldehyde cross linking. Results are shown in Table VII.

TABLE VI

| Sample | Deposition (Percent Wt. of Fabric) |                                      |      | Mols<br>MgCl <sub>2</sub> .6H <sub>2</sub> O<br>per 100 g.<br>Cell | Fabric Properties        |      |            |     |           |
|--------|------------------------------------|--------------------------------------|------|--------------------------------------------------------------------|--------------------------|------|------------|-----|-----------|
|        | DAS                                | MgCl <sub>2</sub> .6H <sub>2</sub> O | HCHO |                                                                    | Percent<br>Bound<br>HCHO | WI%  | CRA° (W+F) |     | Stiffness |
|        |                                    |                                      |      |                                                                    |                          |      | Dry        | Wet |           |
| 1      | 2.5                                | 4.5                                  | 1.85 | 0.0222                                                             | 0.55                     | 51.0 | 223        | 199 | 0.53      |
| 2      | 2.5                                | 5.5                                  | 3.70 | 0.0271                                                             | 0.96                     | 44.4 | 253        | 200 | 0.50      |
| 3      | 2.5                                | 5.5                                  | 5.55 | 0.0271                                                             | 1.36                     | 41.8 | 261        | 217 | 0.50      |
| 4      | 2.5                                | 5.5                                  | 7.40 | 0.0271                                                             | 2.33                     | 35.8 | 277        | 211 | 0.52      |

TABLE VII

| Sample | Additive       | Additive percent | WI%     | Percent Bound HCHO | Pierce bending length after wash No.— |      |      |      |
|--------|----------------|------------------|---------|--------------------|---------------------------------------|------|------|------|
|        |                |                  |         |                    | 0                                     | 1    | 5    | 10   |
| 1      | Starch         | 1                | 50.8    | 0.72               | 0.90                                  | 1.10 | 1.01 | 1.17 |
| 2      | do             | 1                | 37.6    | 1.72               | 1.23                                  | 1.23 | 1.16 | 0.96 |
| 3      | do             | 1                | No HCHO |                    | 1.18                                  | 0.87 | 0.86 | 0.71 |
| 4      | Gelatin        | 1                | 53.8    | 0.87               | 0.89                                  | 1.43 | 1.34 | 1.41 |
| 5      | do             | 1                | 41.6    | 1.82               | 1.48                                  | 1.49 | 1.58 | 1.40 |
| 6      | do             | 1                | No HCHO |                    | 1.12                                  | 0.69 | 0.69 | 0.64 |
| 7      | Polyacrylamide | 1                | 51.0    | 0.71               | 1.68                                  | 1.62 | 1.66 | 1.58 |
| 8      | do             | 1                | 39.5    | 1.84               | 1.65                                  | 1.65 | 1.56 | 1.50 |
| 9      | do             | 1                | No HCHO |                    | 1.51                                  | 0.88 | 0.78 | 0.66 |

We claim:

1. A method for improving the wet and dry crease recovery properties of cellulose fabrics which comprises impregnating said fabrics with formaldehyde, with at least 0.03 mol, per 100 g. of cellulose, of a metallic salt which is a Lewis acid in the solid state and which is water soluble to the extent of at least 0.03 mol/liter at 20° C. and pH 5, and a polymeric film forming stiffening material capable of reacting with formaldehyde, said impregnation with formaldehyde and metallic salt being effected in the presence of water at a pH of at least 5, and curing the impregnated material to cross link the cellulose and to bond the film forming material to the cellulose.

2. The method claimed in claim 1 wherein the metallic salt is magnesium salt.

3. The method claimed in claim 2 wherein the magnesium salt is magnesium chloride.

4. A method for improving the wet and dry crease recovery properties of cellulose fabrics which comprises impregnating said fabrics with formaldehyde, with at least about 0.03 mol, per 100 g. of cellulose, of a salt selected from the group consisting of magnesium chloride, magnesium bromide, magnesium iodide, magnesium nitrate, magnesium perchlorate, zinc nitrate, zinc chloride, zinc sulfate, calcium chloride, calcium bromide, calcium iodide, calcium nitrate, calcium thiocyanate, barium chloride, strontium chloride and cadmium chloride, and with a polymeric film forming stiffening material capable of reacting with formaldehyde, said impregnation with formaldehyde and salt being effected in the presence of water at a pH of at least about 5, and curing the impregnated material to cross-link the cellulose and to bond the stiffening material to the cellulose.

5. A method for improving the dry and wet crease recovery properties of cellulose fabrics which comprises impregnating cellulose fabric with formaldehyde, with at least 0.03 mol, per 100 g. of cellulose, of a salt of a Group II metal and a strong monobasic acid which is at least 50% ionized in normal aqueous solution at 18° C., and with a polymeric film-forming stiffening material, said impregnation with formaldehyde and salt being effected in the presence of water at a pH of at least 5; and curing the impregnated material to cross-link the cellulose and to bond the film forming material to the cellulose.

6. A method for improving the dry and wet crease recovery properties of cellulose fabrics which comprises impregnating said fabrics with formaldehyde, with at least 0.03 mol, per 100 g. of cellulose, of a metallic salt which is a Lewis acid in the solid state and which is water soluble to the extent of at least 0.03 mol/liter at 20° C. and pH 5, and with a polymeric film forming stiffening material selected from the group consisting of starch, starch derivatives, dextran, dextran derivatives, gelatin, natural gums, casein, soybean protein, albumin, algin, polyvinyl alcohol, polyvinyl ethers, polyacrylamide, and cellulose ethers, said impregnation with formaldehyde and metallic salt being effected in the presence of water at a pH of at least about 5, and curing the impregnated material to cross-link the cellulose and to bond the film forming material to the cellulose.

15 7. The method claimed in claim 6 wherein the film forming material is starch.

8. The method claimed in claim 7 wherein the film forming material is gelatin.

9. The method claimed in claim 7 wherein the film forming material is polyvinyl alcohol.

10. The method claimed in claim 7 wherein the film forming material is polyacrylamid.

11. The method claimed in claim 7 wherein the film forming material is dialdehyde starch.

12. A method for improving the wet and dry crease recovery properties of cellulose fabrics which comprises impregnating said fabrics with formaldehyde, with at least 0.03 mol, per 100 g. of cellulose, of a salt of a Group II metal and a strong monobasic acid which is at least 50% ionized in normal aqueous solution at 18° C. and with a polymeric film forming stiffening material selected from the group consisting of starch, starch derivatives, dextran, dextran derivatives, gelatin, natural gums, casein, soybean protein, albumin, algin, polyvinyl alcohol, polyvinyl ethers, polyacrylamide, and cellulose ethers, said impregnation with formaldehyde and salt being effected in the presence of water at a pH of at least about 5, and curing the impregnated material to cross-link the cellulose and to bond the film forming material to the cellulose.

40 13. The method claimed in claim 12 wherein the salt is a magnesium halide.

**14.** The method claimed in claim 13 wherein the salt is magnesium chloride.

45 15. A method for improving the wet and dry crease recovery properties of cellulose fabrics which comprises impregnating said fabrics with formaldehyde, with at least 0.03 mol, per 100 g. of cellulose, of a salt selected from the group consisting of magnesium chloride, magnesium bromide, magnesium iodide, magnesium nitrate, magnesium perchlorate, zinc nitrate, zinc chloride, zinc sulfate, calcium chloride, calcium bromide, calcium iodide, calcium nitrate, calcium thiocyanate, barium chloride, strontium chloride and cadmium chloride, and with a 50 polymeric film forming stiffening material selected from the group consisting of starch, starch derivatives, dextran, dextran derivatives, gelatin, natural gums, casein, soybean protein, albumin, algin, polyvinyl alcohol, polyvinyl ethers, polyacrylamide, and cellulose ethers, said impregnation with formaldehyde and salt being effected in the 55 presence of water at a pH of at least about 5, and curing the impregnated material to cross-link the cellulose and to bond the film forming material to the cellulose.

60

#### References Cited by the Examiner

UNITED STATES PATENTS

- |              |         |             |       |         |
|--------------|---------|-------------|-------|---------|
| 974,488      | 11/1910 | Supf        | ----- | 106—135 |
| 1,506,013    | 8/1924  | Lindauer    | ----- | 106—135 |
| 2,108,520    | 2/1938  | Wolf        | ----- | 8—115.6 |
| 2,238,839    | 4/1941  | Watkins     | ----- | 8—115.6 |
| 70 3,113,826 | 12/1963 | Daul et al. | ----- | 8—116.4 |

NORMAN G. TORCHIN, *Primary Examiner.*

MORRIS O. WOLK, *Examiner.*

75 H. WOLMAN, J. C. CANNON, *Assistant Examiners.*